

Dec. 30, 1952

H. M. HEMMI

2,623,266

CRIMPED FIBERS, FILAMENTS, AND THREADS

Original Filed Nov. 23, 1946

2 SHEETS—SHEET 1

FIG. I



Inventor

Hans Martin Hemmi,

3342 E. F. Wendoroth

Attorney

Dec. 30, 1952

H. M. HEMMI

2,623,266

CRIMPED FIBERS, FILAMENTS, AND THREADS

Original Filed Nov. 23, 1946

2 SHEETS—SHEET 2

FIG. 2



FIG. 3



Inventor

Hans Martin Hemmi,

234

E. F. Wendorff

Attorney

## UNITED STATES PATENT OFFICE

2,623,266

## CRIMPED FIBERS, FILAMENTS, AND THREADS

Hans Martin Hemmi, Basel, Switzerland, assignor  
to Sandoz Ltd., Basel, Switzerland, a Swiss firm

Original application November 23, 1946, Serial No.  
711,928. Divided and this application April 9,  
1948, Serial No. 19,907. In Switzerland De-  
cember 10, 1942

5 Claims. (Cl. 28—81)

1

This application is a division of my patent application Ser. No. 711,928, filed on November 23, 1946, which is a continuation-in-part application of my patent application Ser. No. 514,178 of December 13, 1943, now abandoned.

The present invention relates to a process and to an apparatus for the manufacture of crimped fibres, of all kinds and of any suitable material as stated below having a high crimping degree and which may be destined for further use in view of producing an association of fibres.

With the expression "fibres" reference is also made to filaments, threads and association of "fibres." The materials, of which such fibres are made, may be natural ones, for instance hair, cotton, etc., or synthetic ones such as for instance regenerated cellulose, proteinic fibres, such as lanital, a synthetic high polymeric substance, a thermoplastic material, glass, silicon, metals, natural or artificial silk, etc.

The fibres hitherto known which were crimped in a mechanical manner and which are used as such for the production of an association of fibres always possess sinusoid or spiraloid crimpings. However, it has been found that fibres having a meander-like crimping have a much more wool-like character than fibres with sinusoid or spiraloid crimpings.

The expression "crimping" has a well known technical signification and is determined by the crimping number and crimping degree. The crimping number indicates the number of the crimping present in a length of 1 cm. and is determined on a fibre in unstretched condition by counting the crimping arcs. The crimping degree indicates the relation between the length of a fibre in stretched form and the length of a fibre in unstretched form.

With the expression "meander-like" reference is made to a winding line consisting substantially of circular or nearly circular line portions corresponding to more than half a circle but less than a complete circle and which are joined together in such a manner that there will be turning points between two consecutive circle portions which can lie in the same or in different planes.

The primary object of the present invention is to impart to the fibres or the like to be treated a meander-like crimping by means of an appa-

2

ratus which is fit for this purpose, whereby crimped fibres or the like can be stabilized in their form during or after the crimping operation for instance by means of hardening agents, such as formaldehyde, or by agents to be hardened, for instance watersoluble synthetic resin precondensation products, such as phenoplasts, aminoplasts or alkylol carbamides, like mono- or dimethylol urea, according to the material of which the fibres are made.

Another object of the invention is to realise a process for imparting to the fibres or the like a meander-like crimping.

Another object of the invention is to realise a crimping apparatus with which it is possible to impart to the fibres or the like a meander-like crimping.

Still another object is to realise fibres or the like having a meander-like crimping and being stable to boiling in alkaline soap solutions.

Other objects and advantages of this invention will become apparent from the following description taken in connection with the accompanying drawings, in which:

25 Figure 1 is a longitudinal section of a crimping apparatus of which the middle part is broken out;

Figure 2 is a sectional view taken on the line II—II in Figure 1, and

30 Figure 3 shows, on an enlarged scale, a meander-like fibre produced on the apparatus shown in Figures 1 and 2.

The crimping apparatus according to Figures 1 and 2 has two superposed pairs of link chains 35 *a*, *b* and *c*, *d*, the sprocket wheels *a*<sup>1</sup>, *b*<sup>1</sup> and *c*<sup>1</sup>, *d*<sup>1</sup> of which are fixed on four correspondingly arranged shafts *e*, *f*, *g* and *h*, one of which is extended to one side and forms at the same time the driving shaft of the apparatus. The chain locks of all the link chains are provided with exteriorly projecting supporting arms *a*<sup>2</sup>, *b*<sup>2</sup> *c*<sup>2</sup>, *d*<sup>2</sup> which for corresponding chain locks axially aligned of the chains *a*, *b* or *c*, *d* respectively are interconnected by means of cross bars *m* or *n* respectively of circular cross section. Thus, as can be seen from Figures 1 and 2, the apparatus shown therein, comprises two superposed caterpillar-like chain assemblies the cross bars *m* and *n* which engage each other from opposite sides 45 when the apparatus is running. In this manner

two moving inter-engaged rows of adjacent crimping bars are formed, the outer peripheral portions of which determine a meander-like forming path on which the fibres to be crimped are forced to pass when supplied to the apparatus. The diameter of the cross bars can vary according to the desired crimping number and can for instance be 1.7 mm. It is also possible to vary the depth of the reciprocal engagement of the cross bars by arranging the upper or the lower shafts of the apparatus so that they can be adjusted in vertical direction. The fibres or the like which are to be crimped are supplied to the apparatus from one frontal side of the latter as shown in Figure 1 and are forced to pass through the whole assembly as soon as they are gripped by the first cooperating cross bars *m* and *n*. On their way through the apparatus the fibres will be submitted to the opposite action of the cross bars *m* and *n* which will impart to them a meander-like crimping form as is shown in Figure 1.

The fibres can be natural or synthetic fibres. If it is desired to stabilize the produced crimping, the fibres may be impregnated for instance before passing through the apparatus with a hardening agent or an agent capable of being hardened, the material being hardened either during the passage of the fibres through the apparatus by a heat treatment effected by means of perforated heating tubes *i* (Figure 1) or after having passed the apparatus. If the fibres are made of thermoplastic material, the front part of the apparatus is heated to the necessary temperature, whilst the back part thereof may be cooled, if necessary. The length of the apparatus is so chosen that the fibres are heated during a sufficiently long period and then cooled. For impregnated fibres, which are to be heat-treated during the crimping operation, the apparatus must be so dimensioned that the fibres will leave the apparatus in a hardened condition.

Fibres with meander-like crimpings have in comparison with fibres having a sinusoid or spiraloid crimping the great advantage of having a much more wool-like character and to lose this property to a much smaller extent when washed.

The above used expression "wool-like" is not intended to limit the invention to meander-like crimped fibres which are used for textile purposes. Such fibres can be used in all fields where such an effect is desired.

By the expression "association of fibres" fibres formed for instance by weaving or knitting, such as yarn, cloth or knitted goods are to be understood. The meander-like crimping of the fibres prepared according to the present invention is characterized by the fact that it possesses turning points and further by the relation existing between the distance of the ends of the fibre in crimped and in stretched form. When measured in unstretched condition, the said distance between the ends of the crimped fibres and/or filaments must be less than  $\frac{2}{3}$  of the distance of the fibres ends measured in stretched condition.

In order to fix the meander-like crimping of the fibres the same may be treated in a well-known manner as such or in form of associated fibres with hardening agents, like formaldehyde, or with agents to be hardened, for instance water-soluble synthetic resin precondensation products, such as phenoplasts, aminoplasts or alkylol carbamides, like mono- or dimethylol urea; preferably in presence of catalysts. The material thus treated is then subjected to a heat-

ing operation, e. g. to 100°-150° C., whereby the hardening takes place. After such a treatment the meander-like crimping of the fibres is fixed and becomes stable to boiling.

Figure 3 shows a meander-like crimped fibre produced according to the present invention and the same fibre in stretched state. The distance A to B is less than  $\frac{2}{3}$  of the distance A' to B'.

What I claim is:

1. A new manufactured article made of permanently crimped elongated elements, said elements consisting of organic compounds and being crimped in such a manner that a longitudinal section line therethrough consists of a plurality of successive, interconnected, alternately oppositely directed, essentially circular portions, each of which is more than a semi-circle but less than a complete circle in extent, and the distance between the ends of a crimped element, when measured in plane-projection and in unstretched condition, being less than  $\frac{2}{3}$  of the distance between said ends when measured in stretched condition.

2. A new manufactured article made of permanently crimped cellulose fibres, said fibres containing particles of a hardened synthetic resin as a fixing agent for the crimping and being crimped in such a manner that a longitudinal section line therethrough consists of a plurality of successive, interconnected, alternately oppositely directed, essentially circular portions, each of which is more than a semi-circle but less than a complete circle in extent, and the distance between the ends of a crimped fibre, when measured in plane-projection and in unstretched condition, being less than  $\frac{2}{3}$  of the distance between said ends when measured in stretched condition.

3. A new manufactured article made of permanently crimped cellulose fibres, said fibres containing particles of a hardened synthetic urea-formaldehyde resin as a fixing agent for the crimping and being crimped in such a manner that a longitudinal section line therethrough consists of a plurality of successive, interconnected, alternately oppositely directed, essentially circular portions, each of which is more than a semi-circle but less than a complete circle in extent, and the distance between the ends of a crimped fibre, when measured in plane-projection and in unstretched condition, being less than  $\frac{2}{3}$  of the distance between said ends when measured in stretched condition.

4. A new manufactured article made of permanently crimped synthetic proteinic fibres, said fibres being crimped in such a manner that a longitudinal section line therethrough consists of a plurality of successive, interconnected, alternately oppositely directed, essentially circular portions, each of which is more than a semi-circle but less than a complete circle in extent, and the distance between the ends of a crimped fibre, when measured in plane-projection and in unstretched condition, being less than  $\frac{2}{3}$  of the distance between said ends when measured in stretched condition.

5. A new manufactured article made of permanently crimped hardened synthetic proteinic fibres, said fibres being crimped in such a manner that a longitudinal section line therethrough consists of a plurality of successive, interconnected, alternately oppositely directed, essentially circular portions, each of which is more than a semi-circle but less than a complete circle in extent, and the distance between the ends of a crimped fibre, when measured in plane-projection

and in unstretched condition, being less than  $\frac{2}{3}$  of the distance between said ends when measured in stretched condition.

HANS MARTIN HEMMI.

REFERENCES CITED

The following references are of record in the file of this patent:

UNITED STATES PATENTS

| Number    | Name   | Date          | 10         |
|-----------|--------|---------------|------------|
| 171,357   | Cutter | Dec. 21, 1875 |            |
| 515,891   | Wessel | Mar. 6, 1894  | Number     |
| 642,769   | Wessel | Feb. 6, 1900  | 396,219    |
| 1,186,229 | Ray    | June 6, 1916  | 451,102    |
| 1,427,056 | Breen  | Aug. 22, 1922 | 15 470,601 |

| Number    | Name     | Date          |
|-----------|----------|---------------|
| 2,069,412 | Kronheim | Feb. 2, 1937  |
| 2,208,632 | Dreyfus  | July 23, 1940 |
| 2,251,268 | Clawson  | Aug. 5, 1941  |
| 2,264,978 | Hull     | Dec. 2, 1941  |
| 2,313,630 | Dockerty | Mar. 9, 1943  |
| 2,394,165 | Getaz    | Feb. 5, 1946  |
| 2,508,489 | Browne   | May 23, 1950  |
| 2,601,451 | Page     | June 24, 1952 |

FOREIGN PATENTS

| Number  | Country       | Date          |
|---------|---------------|---------------|
| 396,219 | Great Britain | Aug. 3, 1933  |
| 451,102 | Great Britain | July 7, 1936  |
| 470,601 | Great Britain | Aug. 18, 1937 |